

1

3,232,759  
DIFFUSION TRANSFER PROCESS EMPLOYING  
TONE MODIFIERS

Richard L. White, Edwin B. Wyand, and Hugh G. McGuckin, Rochester, N.Y., assignors to Eastman Kodak Company, Rochester, N.Y., a corporation of New Jersey  
No Drawing. Filed Sept. 13, 1962, Ser. No. 223,532  
14 Claims. (Cl. 96—29)

This invention relates to the production of positive photographic images by the method generally known as the diffusion transfer process, more particularly, a process for improving the tone of the images obtained thereby.

In the diffusion transfer process a light-sensitive silver halide containing emulsion is exposed to light and a negative image formed in the photographic emulsion by developing. A silver solvent is used (generally in the developer) to cause diffusion of the unexposed silver salts onto a receiving sheet held in face contact with the negative. The receiving sheet contains development nuclei which cause the diffused silver salts to form positive silver or silver salt images on the receiving sheet.

A problem encountered in the diffusion transfer process has been that of producing a neutral positive image since the positive image which is often produced is of a brownish or other non-acceptable color. One solution to this problem has been disclosed in U.S. Patent No. 3,004,850, issued to Dickinson et al., October 17, 1961.

It has now been found that a group of compounds can be used either singularly or in combination in small amounts and will produce a shift in the positive image tone toward a neutral color.

One object of this invention is to provide a process for obtaining an improved tone of the positive image obtained in the diffusion transfer process. Another object is to obtain prints by the diffusion transfer process having satisfactory colors. Another object is to obtain the satisfactory neutral color in prints with a short transfer time. An additional object is to provide a group of compounds which can be used either singularly or in combination with an amine-type developer for improving positive image tone.

The above objects are attained by using at least one compound having the general formula:



wherein  $R_1$  and  $R_2$  represent identical alkyl groups such as

Methyl,  
Ethyl,  
Or propyl,

or identical hydroxyalkyl groups such as:

2-hydroxyethyl,  
Or 2-hydroxy-1-propyl,

or, taken together, represent a saturated ring of five or six atoms such as:

Morpholinyl,  
Or piperidyl,

or, if  $R_1$  represents

Hydrogen,  
Or methyl,

$R_2$  represents hydroxyalkyl groups such as:

2-hydroxyethyl,  
1,1-dimethyl-2-hydroxyethyl,

2

1,1-(dihydroxymethyl)-ethyl,  
tris-(hydroxymethyl)-methyl,  
Or glucosyl;

5  $m$  represents a small integer;

$n$  represents an integer between one and six or a fraction representing a mixture of compounds in which  $n$  is between one and six, and

Z represents:

10 Hydrogen,  
Hydrochloride,  
Cyanamide, as the isothiuronium salt,  
Formaldehyde, as a mercaptal,  
Or a metal forming a complex, for instance—  
Silver,  
Zinc,  
Or Zirconium,

20 with an amine-type developer in the diffusion transfer process. The concentration of the above tone modifier is between .01 and 10.0 g. per liter in the developing solution. It will be clear that the developer containing the tone modifier can be applied to the photographic emulsion using the usual means as well as by incorporating it in a pod and squeezing it over the surface of the exposed emulsion.

25 It may also be used in conjunction with the web processing method in which the exposed silver halide emulsion layer containing a latent photographic image is contacted with a hydrophilic organic colloid processing element or web. This processing element contains dispersed silver precipitating agent, and at least at the time of contact with the exposed emulsion layer, sufficient processing solution to develop the exposed silver halide and to remove substantially all of the undeveloped silver halide. For example, a web processing method and composition is disclosed in pending U.S. patent application Serial No. 835,473, filed August 24, 1959, now U.S. Patent 2,960,096.

30 The toning agent may also be coated on the surface of the receiving sheet instead of being placed in the developer itself. The concentration dry basis would be 8 to 80 mg. per square meter on the receiving sheet.

35 The invention includes the process of preparing a direct positive image which comprises exposing a photographic silver halide emulsion layer to an object or image, developing a negative image in the exposed layer, and during or after development, transferring silver halide by diffusion from the unexposed areas of the emulsion layer to a non-light-sensitive image receiving layer containing a silver precipitating agent such as development nuclei or a substance capable of forming development nuclei with dissolved silver halide or a precipitant for silver salts by double decomposition and in effective contact 40 with the emulsion layer, the transfer being effected in the presence of a silver halide solvent and at least one compound of one of the above general formulas.

45 In a preferred embodiment, the silver or zinc salt of the above compounds can be used. For instance, diethylaminoethanethiol HCl can be added to silver nitrate to form the silver salt and added as the silver salt.

50 By "in effective contact" we mean that dissolved silver salts can diffuse from the emulsion layer to the non-light-sensitive layer. There may be an intermediate layer present between the two aforesaid layers which does not hinder the silver salt diffusion, and the two layers may or may not be coated on the same support.

55 Alkaline solution is used to effect development of the exposed layer and the developing agent may be present in either the emulsion layer or in the alkaline solution or both. A mixture of developing agents may be used, if desired.

The silver halide solvent may be present in the developing solution or the receiving layer and is preferably sodium thiosulfate.

It is preferable to employ an antifogant to prevent the formation of fog in the exposed emulsion layer and this may be present in either the emulsion layer or in the alkaline solution used to effect development. Any of the well known nitrogen-containing organic antifogants may be used, or inorganic, such as potassium bromide, which are very suitable.

A suitable known light-insensitive image receiving layer for use in the present invention comprises a gelatin layer containing a substance constituting development nuclei (such as colloidal silver or silver sulfide) or a substance forming development nuclei with dissolved silver salts (such as zinc sulfide), and also containing at least one of the compounds of this invention.

Such a layer may be coated on a paper or film support and contacted in the presence of a silver halide solvent with an exposed and developing emulsion layer which may be coated on a separate support, or may be coated on the same support as the emulsion layer. In the latter, it is preferable to coat the non-light-sensitive layer on a paper support and then to overcoat this layer with a comparatively unhardened emulsion layer. After exposure, development and formation of a direct positive image in the non-light-sensitive layer, the exposed and developed unhardened emulsion layer is removed, for example by washing in warm water. The following examples are intended to illustrate our invention but not to limit it in any way:

*Example 1*

A coating was made on a white, opaque, cellulose acetate support. It was comprised of a 30 mg./ft.<sup>2</sup> nucleated gelatin layer coated over a 1000 mg./ft.<sup>2</sup> gelatin pad. The nuclei were lead sulfide precipitated in 1.5% gelatin.

The web coating was soaked for three minutes in a developer consisting of:

|                                                                          | Grams |
|--------------------------------------------------------------------------|-------|
| 2,2'-iminodietanol-SO <sub>2</sub> addition product, 13% SO <sub>2</sub> |       |
| by weight                                                                | 200.0 |
| 4,4-dimethyl-1-phenyl-3-pyrazolidone                                     | 1.0   |
| Hydroquinone                                                             | 11.0  |
| Sodium thiosulfate                                                       | 8.0   |
| Potassium iodide                                                         | 0.4   |
| Diethylaminoethanethiol HCl                                              | 0.05  |
| 3-mercaptop-1,2,4-triazole                                               | 0.05  |
| Water to make 1 liter.                                                   |       |

The web was removed from the developer, squeegeed, and rolled into contact with an exposed gelatin silver chlorobromide negative film through a pair of wringer rollers. After five minutes the two strips were pulled apart to reveal a fully processed negative and a neutral-toned positive image in the web coating.

When carrying out the process described above, it was found that the second toner by itself gave low maximum densities, but the addition of the diethylaminoethanethiol HCl raised the maximum density considerably.

*Example 2*

A dry processing web was used which consists of a hydrophilic layer comprising, in each square foot, 2 g. gelatin, 8 mg. lead sulfide nuclei, a hardener, and a coating aid coated on polyethylene terephthalate film support. The dry web was soaked for 3 minutes in a developer consisting of:

|                                                                          | Grams |
|--------------------------------------------------------------------------|-------|
| 2,2'-iminodietanol-SO <sub>2</sub> addition product, 13% SO <sub>2</sub> |       |
| by weight                                                                | 200.0 |
| 4-methyl-1-phenyl-3-pyrazolidone                                         | 2.0   |
| Hydroquinone                                                             | 9.0   |
| Sodium thiosulfate, crystalline                                          | 75.0  |
| Diethylaminoethanethiol HCl                                              | 0.5   |
| Water to make 1 liter.                                                   |       |
| Sodium hydroxide to pH 10.00.                                            |       |

The web was removed from the developer and was wound on a spool together with an exposed roll of photographic film having thereon a silver halide emulsion in such a manner that the emulsions of the two strips were in contact. After 10 minutes, the two strips were pulled apart, revealing a neutral tone positive image in the web having a partially fixed negative. After additional fixing, a useable negative obtained, although of low contrast. The addition of diethylaminoethanethiol HCl in this process, by itself produce good neutral tones and density in the web image. Best results were obtained when the negative film was exposed at the recommended film index of 1250.

*Example 3*

15 A processing web was prepared and soaked as in Example 2 except that the amount of diethylaminoethanethiol HCl was 0.75 g. per liter, also, the web-soak time was increased to 5 minutes instead of 3 minutes. Two 20 films were exposed at their recommended exposure indexes of 80 and 200, respectively, and processed by means of the web. After additional fixing, a useable negative of adequate contrast was obtained with both 25 films. The addition of diethylaminoethanethiol HCl, as in Example 2, produced good neutral tones and density in the positive web images.

*Example 4*

30 A processing web was prepared by coating on each square foot of a cellulose acetate support, 2 g. gelatin, 8 mg. lead sulfide nuclei, and 9 mg. diethylaminoethanethiol HCl, together with a hardener and a coating aid.

The web was soaked for 5 minutes in 5 ccs. of the same developer solution used in Example 2 but with the diethylaminoethanethiol HCl omitted. The web was then 35 rolled in contact with an exposed 35 mm. roll of high-speed negative gelatino silver bromoiodide photographic film using a wind-up type processor. After 10 minutes, the film and web were separated.

Neutral tone positive images were obtained in the web 40 after processing.

*Example 5*

45 A receiving sheet was prepared by coating, on each square foot of a white pigmented cellulose acetate support, 1 g. gelatin, 0.45 mg. nickel sulfide nuclei, 260 mg. hypo, 21 mg. 5-diethylaminoethyl-iso-thiuronium chloride HCl, and 0.22 mg. 2 - mercapto - 5 - phenyl - 1,3,4-oxadiazole, together with a hardener and a coating aid.

The receiving sheet and a sheet of exposed, very high-speed negative gelatino silver bromoiodide photographic 50 film were both soaked for 15 seconds in a developer consisting of:

|                                                                          | Grams |
|--------------------------------------------------------------------------|-------|
| 2,2'-iminodietanol-SO <sub>2</sub> addition product, 13% SO <sub>2</sub> | 200.0 |
| Hydroquinone                                                             | 40.0  |
| 4-methyl-1-phenyl-3-pyrazolidone                                         | 0.5   |

After soaking, the two sheets were brought in contact by means of wringer rollers. After 1½ minutes processing time, the strips were pulled apart to reveal a neutral 60 tone positive image in the receiver.

*Example 6*

65 A similar experimental processing web was prepared as used in Example 4 by coating on a white pigmented cellulose acetate support 1 g. gelatin, 500 mg. hypo, and 10 mg. diethylaminoethanethiol HCl per square foot, together with a hardener and a coating aid.

The receiver and an exposed sheet of very high-speed negative gelatino silver bromoiodide photographic film 70 were each soaked for 15 seconds in a developer consisting of:

|                                                                          | Grams |
|--------------------------------------------------------------------------|-------|
| 2,2'-iminodietanol-SO <sub>2</sub> addition product, 13% SO <sub>2</sub> | 100.0 |
| Sodium sulfite                                                           | 75.0  |

|                                  |      |
|----------------------------------|------|
| 2-methylhydroquinone             | 30.0 |
| 4-methyl-1-phenyl-3-pyrazolidone | 0.2  |
| Potassium bromide                | 10.0 |
| Water to make 1 liter.           |      |
| Sodium hydroxide to pH 11.1.     |      |

Processing was carried out as described in Example 5. Neutral tones resulted in the positive image of the receiver.

#### Example 7

A receiver was prepared by coating a layer on white pigmented cellulose acetate support which was comprised of:

|                                                                | Mg./ft. <sup>2</sup> |
|----------------------------------------------------------------|----------------------|
| Gelatin                                                        | 360.0                |
| Sodium sulfite, anhydrous                                      | 25.0                 |
| Sodium thiosulfate, pentahydrate                               | 50.0                 |
| (Ethylenedinitrilo) tetraacetic acid, tetrasodium salt         | 100.0                |
| (Ethylenedinitrilo) tetraacetic acid, trisodium salt           | 200.0                |
| Nickel sulfide nuclei                                          | 0.18                 |
| 1 - methyl - 1,2,3,6 - tetrahydro - 1,3,5 - triazine - 4-thiol | 4.0                  |
| 3,8 - dithiadecane - 1,10 - bis(N - methylpiperidinium pts.)   | 10.0                 |

A hardener and a coating aid were also present in the coating solution. Additional coatings were made containing 0.75, 1.5, 3.0, and 4.5 mg. diethylaminoethanethiol HCl per square foot. The composition of the negative may be summarized as follows:

|                                                                    | Mg./ft. <sup>2</sup> |
|--------------------------------------------------------------------|----------------------|
| Support: Cellulose acetate film with antihalation pelloid backing. |                      |
| Coat 1:                                                            |                      |
| Gelatin                                                            | 250.0                |
| Zinc hydroxide                                                     | 550.0                |
| Coat 2:                                                            |                      |
| Gelatin                                                            | 550.0                |
| Silver bromoiodide (as silver)                                     | 60.0                 |
| 4,4-dimethyl-1-phenyl-3-pyrazolidone                               | 5.0                  |
| Hydroquinone-sulfur dioxide clathrate                              | 33.3                 |
| Coat 3: Gelatin                                                    | 90.0                 |

Sheets of the negative materials were exposed, soaked in tap water for 1 second, and immediately rolled in contact with the sheets of the receiver. After 2 minutes, each pair of sheets was separated.

In the absence of diethylaminoethanethiol HCl, a weak, yellow-brown image was formed in the receiver. The addition of the diethylaminoethanethiol HCl to the extent of 1.5 mg. per square foot shifted the tone to neutral and increased the image density considerably. At the level of 4.5 mg. per square foot, the density was slightly higher. However, the level of 3.0 mg. per square foot was preferred for this particular combination.

#### Example 8

A processing web as described in Example 2 was soaked for 3 minutes in a basic processing solution comprising:

|                                  | Grams per liter |
|----------------------------------|-----------------|
| Hydroquinone                     | 35.0            |
| Sodium sulfite, anhydrous        | 80.0            |
| Sodium thiosulfate, pentahydrate | 15.0            |
| Sodium hydroxide                 | 28.5            |
| Potassium bromide                | 2.5             |
| Benzotriazole                    | 0.12            |

The wet web was squeegeed and rolled in contact with an exposed strip of high-speed reversal type gelatin silver bromoiodide photographic film. After a 5-minute processing period, the strips were separated. The web contained only a faint yellow image.

250 mg. of diethylaminoethanethiol HCl was added per liter of processing solution. A heavy deposit of silver was found in the web indicating the greater efficiency of

75

transfer and toning action over the control. When a similar run was made with the addition of 10 ml. of 2-methylaminoethanol per liter, the tone was more brown than above indicating that the toning action of the diethylaminoethanethiol HCl is more efficient in the presence of an amine.

#### Example 9

A processing web consisting of a cellulose acetate support coated, in each square foot, with a 500 mg. gelatin layer and a 50 mg. gelatin layer containing 0.18 mg. of nickel sulfide nuclei, both layers moderately hardened, was soaked for 10 seconds at 90° F. in a processing solution consisting of:

|    |                                                                                    |    |     |
|----|------------------------------------------------------------------------------------|----|-----|
| 15 | Methyladinoethanol-SO <sub>2</sub> addition product, 20% SO <sub>2</sub> by weight | ml | 160 |
| 16 | Hydroquinone                                                                       | g  | 20  |
| 17 | 1-phenyl-3-pyrazolidone                                                            | g  | 0.5 |
| 18 | Sodium thiosulfate, pentahydrate                                                   | g  | 40  |
| 19 | 20 - 3 - dimethylaminopropylisothiuroniumchloride HCl                              | g  | 0.8 |

Water to make 1 liter.

The web was removed from the processing solution, rolled in contact with a fine-grain silver chlorobromide negative material and allowed to process for 30 seconds in a water bath whose temperature was 90° F. The strips were then separated, revealing blue-black positive image in the web and a developed negative which required an additional fixing treatment. The omission of the 3-dimethylaminopropylisothiuroniumchloride HCl from the processing solution caused the formation of an orange-colored positive in the web. The following structural formula for 3-dimethylaminopropylisothiuroniumchloride HCl:



indicates the reaction which occurs in an alkaline solution. The cyanamide group splits off from the isothiuronium salt leaving the active agent, 3-dimethylaminopropanethiol.

#### Example 10

The processing web of Example 2 was soaked for 3 minutes at room temperature in a processing solution consisting of:

|    | Grams                                                                              |     |
|----|------------------------------------------------------------------------------------|-----|
| 50 | Methylaminoethanol-SO <sub>2</sub> addition product, 20% SO <sub>2</sub> by weight | 100 |
| 51 | Hydroquinone                                                                       | 10  |
| 52 | 4,4-dimethyl-1-phenyl-3-pyrazolidone                                               | 2   |
| 53 | Sodium thiosulfate, pentahydrate                                                   | 130 |
| 54 | 3-dimethylaminopropylisothiuroniumchloride HCl                                     | 0.5 |
| 55 | Water to make 1 liter.                                                             |     |

The web was removed from the processing solution and rolled in contact with an exposed strip of fine-grain silver bromoiodide negative material in such a manner that the two emulsions were in contact. After 10 minutes of transfer at room temperature the strips were pulled apart, revealing a neutral tone positive image in the web and a completely fixed negative.

#### Example 11

A processing solution was prepared containing a low polymer of alkylaminoalkanethiol, 2-hydroxy-1,1-dimethylaminooxyethylenesulfide-1,69



This processing solution consisted of:

|                                                                          | Grams |
|--------------------------------------------------------------------------|-------|
| Methylaminoethanol-SO <sub>2</sub> addition product, 20% SO <sub>2</sub> |       |
| by weight                                                                | 100   |
| Hydroquinone                                                             | 10    |
| 4,4-dimethyl-1-phenyl-3-pyrazolidone                                     | 2     |
| Sodium thiosulfate, pentahydrate                                         | 130   |
| 1,1-dimethyl - 2 - hydroxyethylaminooligoethylene-<br>sulfide-1.69       | 0.75  |
| Water to make 1 liter.                                                   |       |

The web of Example 2 was soaked in the solution for 3 minutes, removed and rolled in contact with an exposed strip of a fine-grain silver bromoiodide negative material in such a manner that the two emulsions were in contact. After ten minutes of transfer at room temperature, the strips were pulled apart, revealing a blue-black positive image in the web and a completely fixed negative. When the toning agent was omitted from the processing solution, a brown image was formed in the web.

For the oligomeric compounds of the type used in Example 11, higher degrees of polymerization were also effective, as in the case of 1,1-dimethyl-2-hydroxyethylaminooligoethylene sulfide-2.9.



*Example 12*

An experimental processing web like that of Example 2 was soaked for ten seconds at 90° F. in a processing solution consisting of:

|                                                                          |           |
|--------------------------------------------------------------------------|-----------|
| Methylaminoethanol-SO <sub>2</sub> addition product, 20% SO <sub>2</sub> |           |
| by weight                                                                | ml. 160   |
| Hydroquinone                                                             | grams 20  |
| 1-phenyl-3-pyrazolidone                                                  | do 0.5    |
| Sodium thiosulfate, pentahydrate                                         | do 40     |
| 1,1-dimethyl-2-hydroxyethylaminooligoethylene sul-<br>fide-2.9           | grams 0.2 |
| Water to make 1 liter.                                                   |           |

The web was removed from the processing solution, rolled in contact with the negative material of Example 9, and allowed to process for 30 seconds in a water bath whose temperature was 90° F. The strips were then separated, revealing a blue-black positive image of good density in the web and a developed negative which required an additional fixing treatment. Orange tones were obtained in the positive image in the web when the toner was omitted from the processing solution.

*Example 13*

A web like that of Example 9 was soaked for ten seconds at 90° F. in a processing solution consisting of:

|                                                                    |          |
|--------------------------------------------------------------------|----------|
| Methylaminoethanol                                                 | ml. 50   |
| Sodium sulfite, anhydrous                                          | grams 20 |
| Hydroquinone                                                       | do 20    |
| 4,4-dimethyl-1-phenyl-3-pyrazolidone                               | do 2     |
| Sodium thiosulfate, pentahydrate                                   | do 30    |
| Sulfuric acid to pH of 10.0.                                       |          |
| 1,1 - dimethyl - 2 - hydroxyethylaminooligoethylene<br>sulfide-2.9 | gram 0.5 |
| Water to make 1 liter.                                             |          |

The web was removed from the processing solution, rolled in contact with a moderate-speed silver bromoiodide negative material, and allowed to process for 60 seconds in a water bath whose temperature was 90° F. The strips were then separated revealing a blue-black positive image in the web and a developed negative which required an additional fixing treatment.

A combination of the toner 1,1-dimethyl-2-hydroxyethylaminooligoethylene sulfide-2.9 and diethylaminoethanethiol HCl was found to be particularly effective in the photographic system of Example 7.

*Example 14*

The negative of Example 7 was exposed and soaked in tap water for six seconds. It was then rolled in contact with a receiver which was prepared by coating a layer on white-pigmented cellulose acetate support which was comprised of:

|                                                                | Mg./ft. <sup>2</sup> |
|----------------------------------------------------------------|----------------------|
| Gelatin                                                        | 360.0                |
| Sodium sulfite, anhydrous                                      | 25.0                 |
| Sodium thiosulfate, pentahydrate                               | 50.0                 |
| Ethylenediaminetetraacetic acid, tetrasodium salt              | 100.0                |
| Ethylenediaminetetraacetic acid, trisodium salt                | 200.0                |
| Nickel sulfide nuclei                                          | 0.14                 |
| Diethylaminoethanethiol HCl                                    | 19.2                 |
| Sulfuric acid to pH of 10.0.                                   |                      |
| 1,1-dimethyl-2-hydroxyethylaminooligoethylene sul-<br>fide-2.9 | gram 0.5             |

together with a hardener and a coating aid. After two minutes, the two sheets were separated. The receiver contained a high-density, neutral-toned positive image.

Other compounds similar to 2-hydroxy-1,1-dimethyl-ethylaminooligoethylene sulfide-1.69 and 1,1-dimethyl-2-hydroxyethylaminooligoethylene sulfide-2.9 were found to be effective in combination with diethylaminoethanethiol HCl in the system of Example 14.

2-hydroxyethylaminooligoethylene sulfide-1



|      |                                                       |
|------|-------------------------------------------------------|
| 30   | 1,1-(dihydroxymethyl)ethylaminooligoethylene sulfide- |
| 3.43 |                                                       |



|      |                                                       |
|------|-------------------------------------------------------|
| 4.88 | Tris - hydroxymethylmethylaminooligoethylene sulfide- |
| 40   |                                                       |



|      |                                                         |
|------|---------------------------------------------------------|
| 3.47 | Bis(2 - hydroxy - 1-propyl)aminoooligoethylene sulfide- |
| 45   |                                                         |



N-methylglucaminooligoethylene sulfide-5.6

|    |                                                                                                             |
|----|-------------------------------------------------------------------------------------------------------------|
| 50 | HOCH <sub>2</sub> (CHOH) <sub>4</sub> CH <sub>2</sub> N(CH <sub>2</sub> CH <sub>2</sub> S) <sub>5.6</sub> H |
| 55 |                                                                                                             |

|    |                                                                     |
|----|---------------------------------------------------------------------|
| 55 | N - (2-aminoethyl)-2-hydroxyethylaminooligoethylene<br>sulfide-1.75 |
| 60 |                                                                     |



Morpholinoethanethiol



|    |                                                               |
|----|---------------------------------------------------------------|
| 65 | 2 - morpholinoethylisothiuronium, chloride hydrochlo-<br>ride |
| 70 |                                                               |



*Example 15*

Strips of a negative like that described in Example 7 were exposed, soaked for six seconds in water or a solution comprising 0.75 gram of diethylaminoethanethiol HCl per liter, and then placed in contact with a receiver

like that of Example 14 except that the toners were omitted. The receiver images had the following appearance:

| Solution                     | Transfer time | Receiver image appearance |
|------------------------------|---------------|---------------------------|
| Water                        | 2 min         | Orange.                   |
| Diethylaminoethanethiol HCl. | 2 min         | Weak brown.               |
| Do                           | 3 min         | Neutral, high density.    |

#### Example 16

A negative whose composition may be summarized as follows:

Support: Cellulose acetate film with antihalation pellloid backing.

Coat 1:

|                | Mg./ft. <sup>2</sup> | Grams                                                                    |
|----------------|----------------------|--------------------------------------------------------------------------|
| Gelatin        | 250.0                | Methylaminoethanol-SO <sub>2</sub> addition product, 19% SO <sub>2</sub> |
| Zinc hydroxide | 550.0                | by weight                                                                |

Coat 2:

|                                       |       |
|---------------------------------------|-------|
| Gelatin                               | 275.0 |
| Silver bromoiodide (as silver)        | 60.0  |
| 4,4-dimethyl-1-phenyl-3-pyrazolidone  | 11.0  |
| Hydroquinone-sulfur dioxide clathrate | 33.3  |

Coat 3: Gelatin 90.0

was exposed and soaked for six seconds in a solution containing approximately 500 mg. diethylaminoethanethiol and 200 mg. 1,1-dimethyl-2-hydroxymethylaminoolefin-ethylene sulfide-2.9 per liter. Both compounds were present in the solution as silver complex salts, formed by combining one mole of silver nitrate with two moles of the organic compound. The formation of a tightly-bound complex was indicated by the disappearance of the characteristic odor of each compound. After soaking, the negative was rolled in contact with a receiver like that of Example 14 but from which the toners had been omitted. After three minutes, the two sheets were separated, revealing a neutral-toned positive image in the receiver.

#### Example 17

The experiment of the preceding example was repeated with the water for soaking the negative containing 0.5 gram of 2-dimethylaminoethylmercapto zinc chloride hydrochloride and 2.0 grams of 2-morpholinoethylisothiuronium chloride hydrochloride per liter. A neutral-toned positive image was obtained.

#### Example 18

Processing web A was prepared which comprised, per square foot, 2000 mg. gelatin, nickel sulfide nuclei, 12 mg. diethylaminoethanethiol, a hardener and a coating aid, coated on a polyethylene terephthalate support. In a second web, B, the 12 mg. of diethylaminoethanethiol had previously been combined with 6 mg. of silver nitrate. The webs were soaked for periods of time ranging from 1½ to 12 minutes at 70° F. in a processing solution comprising:

|                                                             | Grams |
|-------------------------------------------------------------|-------|
| 2,2'-iminodiethanol-SO <sub>2</sub> addition product, 12.8% |       |
| SO <sub>2</sub> by weight                                   | 200   |
| 4,4-dimethyl-1-phenyl-3-pyrazolidone                        | 2     |
| Hydroquinone                                                | 40    |
| Sodium thiosulfate, pentahydrate                            | 100   |
| Sodium hydroxide to pH 10.5.                                |       |
| Water to make 1 liter.                                      |       |

and placed in contact with exposed strips of a fine-grain gelatino silver bromoiodide negative for ten minutes.

The negatives for both webs showed only a slight increase in speed and contrast as the web soak time was increased. The positive images in Web A showed a progressive lowering of contrast, as represented by a lengthening of the toe and a falling off of the shoulder, as the soak time was increased. The shape and position of the positive curve in Web B was not influenced by the length of

the soak period. It was evident that the diethylaminoethanethiol was slowly washed out of Web A during the soaking period, while, as the silver salt in Web B, the loss of the compound was eliminated or at least greatly reduced.

#### Example 19

Processing webs like those of Example 18 above were prepared in which Web C contained no toning agent and Web D contained 4 mg. of diethylaminoethanethiol per square foot complexed with 2 mg. of silver nitrate. Samples of the two webs were incubated for one week at 100° F. and 80 percent relative humidity. The incubated and non-incubated webs were soaked for 4 minutes at 70° F. in a solution comprised of:

|                                                                          | Grams |
|--------------------------------------------------------------------------|-------|
| Methylaminoethanol-SO <sub>2</sub> addition product, 19% SO <sub>2</sub> |       |
| by weight                                                                | 100   |
| Dimezone                                                                 | 2     |
| Hydroquinone                                                             | 10    |
| 20 Sodium thiosulfate, pentahydrate                                      | 100   |
| Ethanol                                                                  | 100   |
| Water to make 1 liter.                                                   |       |

and placed in contact with exposed strips of a fine-grain gelatino silver bromoiodide negative material for ten minutes. Incubation of the processing webs caused the positive image curves to be shifted in a direction representing a higher sensitometric speed. In the absence of the diethylaminoethanethiol-silver salt, the shift amounted to 0.36 log E at a density of 1.0, while in the presence of the diethylaminoethanethiol-silver salt, the shift was only 0.07 log E. The diethylaminoethanethiol-silver salt evidently stabilized the nuclei to high humidity incubation, presumably by adsorption on the nuclei. Other experiments had shown that diethylaminoethanethiol would become degraded or sublime from a coating under conditions of high temperature or moist incubation unless complexed as a metal salt, an isothiuronium salt, a mercaptal, or the like.

#### Example 20

Processing Web A is prepared as described in Example 18 except that in the second web, B, the 12 mg. of diethylaminoethanethiol is combined with 6 mg. of zinc nitrate. The webs are soaked for periods of time ranging from 1½ to 12 minutes at 70° F. in the processing solution described in Example 18, and placed in contact with exposed strips of a fine-grain gelatino silver bromoiodide negative for ten minutes.

The negatives for both webs show only a slight increase in speed and contrast as the web soak time was increased. The positive images in Web A show a progressive lowering of contrast as represented by a lengthening of the toe and a falling off of the shoulder, as the soak time is increased. The shape and position of the positive curve in Web B is not influenced by the length of the soak period. It is evident that the diethylaminoethanethiol is slowly washed out of Web A during the soaking period, while, as the zinc salt in Web B, the loss of the compound is eliminated or least greatly reduced.

#### Example 21

An extremely useful attribute of diethylaminoethanethiol is the ability to markedly reduce the time required to form a full-density, neutral-toned positive transfer image. In equivalent transfer systems, one or two minutes of contact with the negative are necessary for complete transfer. At shorter times the positive is orange or brown colored and of low density. In the presence of diethylaminoethanethiol the same amount of transfer can take place in 15 or 20 seconds. The effect was observed in a diffusion transfer system containing a toning agent combination disclosed and claimed in the Tregillus et al. U.S. Patent No. 3,017,270 as extended by the U.S. patent application Ser. No. 141,036, filed September 27, 1961 and now abandoned, by A. A. Rasch, P. B. Gilman, and J. E. Jones.

A fine-grain gelatino silver bromoiodide negative film was exposed and then dipped for six seconds at 70° F. in a solution comprising:

|                                                             | Grams |
|-------------------------------------------------------------|-------|
| 2,2'-iminodiethanol-SO <sub>2</sub> addition product, 12.8% |       |
| SO <sub>2</sub> by weight                                   | 160.0 |
| Methylaminoethanol-SO <sub>2</sub> addition product, 19%    |       |
| SO <sub>2</sub> by weight                                   | 20.0  |
| 1-phenyl-3-pyrazolidone                                     | 1.0   |
| Hydroquinone                                                | 12.0  |
| Sodium thiosulfate, pentahydrate                            | 60.0  |
| Triton X-200 (surfactant)                                   | 0.5   |
| Sodium hydroxide to pH 10.5.                                |       |
| Water to make 1 liter.                                      |       |

As Run A, the negative was immediately placed in contact for 20 seconds at 70° F. with a receiver consisting of a white-pigmented at 70° F. with a receiver consisting of coated, per sq. ft., 1000 mg. gelatin, 0.3 mg. nickel sulfide nuclei, a hardener, and a coating aid.

Run A was repeated with the following changes:

Run B.—2.0 grams per liter of 3,8-dithiadecane-1,10-bis(N-methylpiperidinium-p-toluene sulfonate) were added to the processing solution.

Run C.—0.1 gram of 1-methyl-1,2,3,6-tetrahydro-1,3,5-triazine-4-thiol were added to one liter of the processing solution.

Run D.—The additions of Runs B and C were combined.

Run E.—The negative was dipped in the solution of Run D and placed in contact with a receiver containing, in addition, a complex formed by combining 4 mg. of diethylaminoethanethiol and 2 mg. of silver nitrate.

The positive images in the receivers of the various runs were found to possess the following characteristics:

| Run | Image color  | Maximum density |
|-----|--------------|-----------------|
| A   | Orange       | 0.89            |
| B   | Orange-brown | 0.98            |
| C   | Orange       | 0.90            |
| D   | Orange-brown | 0.94            |
| E   | Near-neutral | 1.37            |

Subsequently, the receiver and processing solution were modified slightly and rebalanced so that the image tone was substantially neutral and the maximum density was on the order of 1.6.

Polymeric sulfides described as useful in this invention are described in pending U.S. patent application 165,931, filed January 12, 1962 and now abandoned, in the names of Johnson and Reynolds.

The invention has been described in detail with particular reference to preferred embodiments thereof, but it will be understood that variations and modifications can be effected within the spirit and scope of the invention as described hereinabove and as defined in the appended claims.

We claim:

1. A process for preparing a photographic image which comprises developing an exposed photographic silver halide emulsion layer with a silver halide developing agent and transferring the silver halide by diffusion from the undeveloped areas of the emulsion layer to a supported image receiving layer containing development nuclei, transfer being effected in contiguity with sufficient silver halide solvent to remove substantially all undeveloped silver halide from the emulsion layer, an alkanolamine and, in addition, a toning compound, said compound being different from the silver halide solvent, having the general formula:



wherein R<sub>1</sub> and R<sub>2</sub> are selected from the class consisting

of H, lower alkyl, lower hydroxyalkyl and non-metallic atoms necessary to complete a heterocyclic ring selected from the class consisting of morpholinyl and piperidyl, m represents a number of 1-3, n represents a number between 1 and 6 and Z represents a member selected from the class consisting of hydrogen, iminocarbamoyl, hydroxymethyl, silver, zinc and zirconium.

2. The process of claim 1 wherein the toning compound is incorporated in the developer solution.

3. The process of claim 1 wherein the toning compound is incorporated in the image receiving layer.

4. A process for preparing a photographic image which comprises developing an exposed photographic silver halide emulsion layer with a silver halide developing agent and transferring the silver halide by diffusion from the undeveloped areas of the emulsion layer to a supported image receiving layer containing development nuclei, the transfer being effected in contiguity with sufficient silver halide solvent, other than diethylaminoethane-thiol HCl, to remove substantially all undeveloped silver halide from the emulsion layer, an alkanolamine and, in addition, diethylaminoethanethiol HCl.

5. A process for preparing a photographic image which comprises developing an exposed photographic silver halide emulsion layer with a silver halide developing agent and transferring the silver halide by diffusion from the undeveloped areas of the emulsion layer to a supported image receiving layer containing development nuclei, the transfer being effected in contiguity with sufficient silver halide solvent to remove substantially all undeveloped silver halide from the emulsion layer, an alkanolamine and, in addition, 2-hydroxyethylamino-oligoethylene sulfide.

6. A process for preparing a photographic image which comprises developing an exposed photographic silver halide emulsion layer with a silver halide developing agent and transferring the silver halide by diffusion from the undeveloped areas of the emulsion layer to a supported image receiving layer containing development nuclei, the transfer being effected in contiguity with sufficient silver halide solvent to remove substantially all undeveloped silver halide from the emulsion layer, an alkanolamine and, in addition, 2-hydroxy-1,1-dimethyl-ethylaminooligoethylene sulfide.

7. A process for preparing a photographic image which comprises developing an exposed photographic silver halide emulsion layer with a silver halide developing agent and transferring the silver halide by diffusion from the undeveloped areas of the emulsion layer to a supported image receiving layer containing development nuclei, the transfer being effected in contiguity with sufficient silver halide solvent to remove substantially all undeveloped silver halide from the emulsion layer, an alkanolamine and, in addition, morpholinoethanethiol.

8. A process for preparing a photographic image which comprises developing an exposed photographic silver halide emulsion layer with a silver halide developing agent and transferring the silver halide by diffusion from the undeveloped areas of the emulsion layer to a supported image receiving layer containing development nuclei, the transfer being effected in contiguity with sufficient silver halide solvent to remove substantially all undeveloped silver halide from the emulsion layer, an alkanolamine and, in addition, 1,1-(dihydroxymethyl)-ethylaminooligoethylene sulfide.

9. A process for preparing a photographic image which comprises developing an exposed photographic silver halide emulsion layer with a silver halide developing agent and transferring the silver halide by diffusion from the undeveloped areas of the emulsion layer to a supported image receiving layer containing development nuclei, the transfer being effected in contiguity with sufficient silver halide solvent to remove substantially all undeveloped silver halide from the emulsion layer, an

alkanolamine and, in addition, tris-hydroxymethylmethylaminoaligoethylene sulfide.

10. A process for preparing a photographic image which comprises developing an exposed photographic silver halide emulsion layer with a silver halide developing agent and transferring the silver halide by diffusion from the undeveloped areas of the emulsion layer to a supported image receiving layer containing development nuclei, the transfer being effected in contiguity with sufficient silver halide solvent to remove substantially all undeveloped silver halide from the emulsion layer, an alkanolamine and, in addition, bis(2-hydroxy-1-propyl)aminoaligoethylene sulfide.

11. A process for preparing a photographic image which comprises developing an exposed photographic silver halide emulsion layer with a silver halide developing agent and transferring the silver halide by diffusion from the undeveloped areas of the emulsion layer to a supported image receiving layer containing development nuclei, the transfer being effected in contiguity with sufficient silver halide solvent to remove substantially all undeveloped silver halide from the emulsion layer, an alkanolamine and, in addition, N-methylglucaminoaligoethylene sulfide.

12. A process for preparing a photographic image which comprises developing an exposed photographic silver halide emulsion layer with a silver halide developing agent and transferring the silver halide by diffusion from the undeveloped areas of the emulsion layer to a supported image receiving layer containing development nuclei, the transfer being effected in contiguity with sufficient silver halide solvent to remove substantially all undeveloped silver halide from the emulsion layer, an alkanolamine and, in addition, N-(2-aminoethyl)-2-hydroxyethylaminoaligoethylene sulfide.

13. A process for preparing a photographic image which comprises developing an exposed photographic sil-

ver halide emulsion layer with a silver halide developing agent and transferring the silver halide by diffusion from the undeveloped areas of the emulsion layer to a supported image receiving layer containing development nuclei, the transfer being effected in contiguity with sufficient silver halide solvent to remove substantially all undeveloped silver halide from the emulsion layer, an alkanolamine and, in addition, the silver salt of diethylaminoethanethiol HCl.

14. A process for preparing a photographic image which comprises developing an exposed photographic silver halide emulsion layer with a silver halide developing agent and transferring the silver halide by diffusion from the undeveloped areas of the emulsion layer to a supported image receiving layer containing development nuclei, the transfer being effected in contiguity with sufficient silver halide solvent to remove substantially all undeveloped silver halide from the emulsion layer, an alkanolamine and, in addition, the zinc salt of diethylaminoethanethiol HCl.

20

#### References Cited by the Examiner

##### UNITED STATES PATENTS

|    |           |         |              |       |       |
|----|-----------|---------|--------------|-------|-------|
| 25 | 2,698,245 | 12/1954 | Land         | ----- | 96—29 |
|    | 2,875,048 | 2/1959  | Haist et al. | ----- | 96—61 |
|    | 2,984,565 | 5/1961  | Morse        | ----- | 96—29 |
|    | 3,017,270 | 1/1962  | Tregillus    | ----- | 96—29 |

##### FOREIGN PATENTS

|    |           |                |
|----|-----------|----------------|
| 30 | 594,237   | Belgium.       |
|    | 1,243,430 | 9/1960 France. |

##### OTHER REFERENCES

Photographic Science and Engineering, 5, July—August 35 1961, pp. 198—203.

NORMAN G. TORCHIN, *Primary Examiner.*